

## UNITED STATES PATENT OFFICE

JACK ROBINSON, OF WOOD RIVER, ILLINOIS, ASSIGNOR TO STANDARD OIL COMPANY, OF WHITING, INDIANA, A CORPORATION OF INDIANA

## LUBRICATING OIL

No Drawing.

Application filed June 30, 1927. Serial No. 202,758.

This invention relates to lubricating oils and particularly to oils for lubricating turbines and similar purposes.

When ordinary lubricating oils are used in steam turbines, they readily form objectionable quantities of sludge. In order to avoid this objectionable characteristic, it has become the practice to employ as turbine oils, lubricating oils which have been drastically treated with strong or fuming sulphuric acid to remove coloring matter and large percentages of other constituents, to give a so-called "white oil." These highly treated oils are, however, subject to the further disadvantage that, after a relatively short period of use, they form acidic oxidation products and form emulsions from which the oil is separable only with difficulty.

The basis of the present invention is the discovery that by subjecting the lubricating oil to treatment with a certain, relatively small, critical amount of sulphuric acid, a much more satisfactory turbine oil possessing much greater resistance to oxidation and retaining great demulsibility, results.

As stated, the amount of the acid used for the treatment is critical and will vary for various oils, the nature of the acid employed and other factors. Accordingly, the invention will be described by reference to a particular oil and particular tests will be described, by means of which, the critical treatment for any particular oil may be determined.

For this purpose the following specific example is given.

Fifteen gallons of mid-continent distillate lubricating oil of 296 seconds viscosity at 100° F. are mixed with five gallons of a similar distillate of 100 seconds viscosity at 100° F. to give a mixture of 235 seconds viscosity at 100° F. A half pound of fuming acid per gallon of the original charge is applied at intervals of twenty-four hours, and the batch given an air blow of from twenty to one hundred minutes. The batch is allowed to settle over night and the sludge withdrawn. The acid supplied each day is based upon the original oil treated, disregarding treating losses but taking into

account the samples removed daily. This is continued for eleven dumps so that the amount of fuming acid supplied is 5½ pounds per gallon of the original oil. The sludge loss during this period amounts to about 65% of the original oil. About 15% loss is incurred after the first dump, about 8% after each of the second and third dumps, about 6½% after each of the fourth and fifth dumps, and about 4½% after each of the sixth and seventh dumps.

Each sample withdrawn is blown for about one hour at a temperature of between 140° and 160° F. The sour oil is neutralized with caustic soda in excess and kept at 160° F., the caustic soda is withdrawn, and the oil given two alcohol washes and a water wash followed by blowing until free from water. The sample is then filtered through clay, and subjected to an oxidation test.

The method of conducting this test is to subject a sample of the oil to oxidation conditions which simulate as far as possible the oxidation conditions to which turbine oil is subjected during use and to determine the acidity and demulsibility (Herschel) after a certain time.

A suitable oxidation test is to pass oxygen through a sample of the oil maintained at about 212° F. for a long period. It has been found that the oxidation ordinarily has a slight effect at first, but that the rate of oxidation increases rapidly with time. A suitable period of time in which the course of oxidation is shown unmistakably is about three hundred hours.

The following results have been obtained:

| Fuming acid pounds per gallon | Acidity mg. KOH per gal. of oil after 300 hrs. test | Demulsibility (Herschel) after 300 hrs. test |
|-------------------------------|-----------------------------------------------------|----------------------------------------------|
| 1                             | .0695                                               | 60                                           |
| 2                             | .0135                                               | 1620                                         |
| 3                             | .0110                                               | 1300                                         |
| 4.5                           | 26.8                                                | 720                                          |
| 5.5                           | 23.5                                                | 780                                          |

The demulsibility test employed in testing the above samples was the (Herschel) test No. 320.31 described in Technical Pa- 100

per (323-b), Bureau of Mines, 1927, on page 85. This test is made at a temperature of 130° F. with 27 cc. sample and the basis for determining the maximum rate of demulsibility is one hour. Thus, the maximum possible demulsibility is 1620.

It is remarkable that the oil treated with 4.5 and 5.5 pounds of acid per gallon develops large acidities and that immediately 10 below this point, that is, oil treated with two or three pounds of acid per gallon, practically no acidity develops. As to demulsibility, in the presence of the large amounts of acid produced in the oils treated with 15 4.5 and 5.5 pounds per gallon, soaps would form with the metal of the turbine and reduce the demulsibility of these oils greatly below the figures shown above; for example the demulsibility would be 20 reduced substantially below 150 under these circumstances.

Thus, it is clear that by treatment with a certain critical amount of acid with the particular oil, acid and conditions indicated 25 above said amount being about two or three pounds per gallon in the case set forth, there results a turbine oil of remarkable properties, such oil developing practically no acidity and retaining demulsibility of very high 30 order after protracted exposure to turbine operating conditions.

Although the present invention has been described in connection with the details of a specific example thereof, it is not intended 35 that such details shall be regarded as limitations upon the scope of the invention, except in so far as included in the accompanying claims. In particular, it is pointed out that it is impossible to state definitely the extent of the critical amount of acid necessary 40 for treatment of different oils under different conditions. Applicant has, however discovered that there is a certain critical amount of acid which yields oils of remarkable 45 properties and utility, and has clearly shown how such critical amount may be determined for any particular oil. It is to be understood that the expression "critical amount" used in the appended claims is intended to designate that particular amount 50 of acid which yields oils which are strongly resistant to oxidation and retain high demulsibility after treatment to turbine operation oxidation conditions, for prolonged 55 periods, such as are exemplified by the oils described above which have been treated with two or three pounds of fuming sulphuric acid per gallon.

I claim:

60 1. The method of producing turbine oils which consists in subjecting lubricating oils to treatment with a critical amount of sulphuric acid of a strength at least equal to that of concentrated sulfuric acid, calculated to render it remarkably resistant to oxidation 65

and retain high demulsibility when subjected to turbine oxidation conditions for a prolonged period.

2. The method of producing turbine oils which consists in subjecting a lubricating oil 70 to repeated treatments with sulfuric acid of a strength at least equal to that of concentrated sulfuric acid, taking samples of the oil treated with different amounts of said sulfuric acid, finishing said samples, and subjecting them for a long period to oxidation treatment resembling the conditions in an operating turbine, determining the acidity and demulsibility of the oxidized samples, and treating the bulk of the oil with the 75 amount of said sulfuric acid which corresponds with the amount of said sulfuric acid used in the treatment of a sample which gives a low acidity and high demulsibility 80 after said oxidation test.

3. The method of producing turbine oils which consists in subjecting a lubricating oil to a treatment with fuming sulphuric acid to the extent of about two to three pounds per gallon to render it remarkably resistant to 85 oxidation and retain high demulsibility when subjected to turbine oxidation conditions for a prolonged period.

4. The method of producing turbine oils which consists in subjecting a lubricating oil 90 to repeated treatments with fuming sulfuric acid, taking samples of the oil treated with different amounts of fuming sulfuric acid, finishing said samples, and subjecting them for a long period to oxidation treatment resembling the conditions in an operating turbine, determining the acidity and demulsibility of the oxidized samples, and treating the bulk of the oil with the amount of fuming sulfuric acid which corresponds with 95 the amount of fuming sulfuric acid used in the treatment of a sample which gives a low acidity and high demulsibility after said oxidation test.

5. The method of producing turbine oils 100 which consists in treating various samples of a given bulk of lubricating oil with various amounts of fuming sulfuric acid to determine the critical amount of sulphuric acid 105 calculated to render it remarkably resistant to oxidation and retain high demulsibility when subjected to turbine oxidation conditions for a prolonged period, and treating the bulk of the lubricating oil with the critical amount of fuming sulfuric acid so determined.

6. The method of producing turbine oils which consists in subjecting a lubricating oil to a treatment with sulphuric acid of a 110 strength at least equal to that of concentrated sulphuric acid to the extent of about two to three pounds per gallon to render it remarkably 115 resistant to oxidation and retain high demulsibility when subjected to turbine oxidation conditions for a prolonged period.

7. The method of producing turbine oils which consists in treating various samples of a given bulk of lubricating oil with various amounts of sulphuric acid of a strength at least equal to that of concentrated sulfuric acid to determine the critical amount of sulphuric acid calculated to render it remarkably resistant to oxidation and retain high demulsibility when subjected to turbine oxidation conditions for a prolonged period, and treating the bulk of the lubricating oil with the critical amount of strong sulphuric acid so determined.

In witness whereof, I have hereunto set my hand, this 10th day of June, 1927.

JACK ROBINSON.

20

25

30

35

40

45

50

55

60

65